

## METHOD OF TANNING HIDE

Richard W. Alsgaard and John W. Gilkey, Midland, Mich., assignors to Dow Corning Corporation, Midland, Mich., a corporation of Michigan

No Drawing. Filed Dec. 15, 1958, Ser. No. 780,229

2 Claims. (Cl. 8—94.33)

This invention relates to a novel method of preparing leather by tanning hides with certain organosilicon compounds.

The principal commercial methods of tanning leather such as chrome tannage and vegetable tannage produce leathers which are colored. Consequently, in order to prepare white leather articles from leather that has been so tanned it is necessary to employ bleaching agents and large quantities of white pigments such as titanium dioxide. These pigments cover up the color of the leather.

Ordinarily such white leather functions satisfactorily for most applications. However, it has been impossible to render the presently available commercial white leather water repellent with silicones. Inasmuch as silicone water repellents are highly desirable for use on leather, the inability to water repel present commercial white leathers has been a disadvantage. For example, nurses' shoes are often in contact with water borne materials which are deleterious to leather. It would be highly desirable, therefore, if silicone water repellents could be satisfactorily applied to such shoes. However, to date, this has not been feasible.

It is the object of this invention to provide a novel procedure for tanning leather. Another object is to provide a white leather which can be made water repellent with commercial silicone water repellents. Other objects and advantages will be apparent from the following description.

This invention relates to a method of preparing leather which comprises contacting hide with an aqueous dispersion of an organosilicon compound of the formula



in which R is an aliphatic hydrocarbon radical of less than 4 C atoms and n is an integer of from 2 to 3 inclusive, said dispersion having a pH of at least 9 until the hide is suitably tanned, the organosilicon compound being present in amount of at least 10% of the dry weight of the hide.

In carrying out the process of this invention the hide can be contacted with the aqueous dispersion of the organosilicon compound in any desired manner. The aqueous dispersion can be either in the form of a solution of the organosilicon compound or an emulsion thereof. In general, the preferred method is to immerse the hide in the aqueous dispersion and agitate the mixture until the hide is suitably tanned. The time of tanning is not critical and, in general, satisfactory results are obtained after the hide has been in contact with the dispersion for from 10 to 24 hours. It should be understood, of course, that shorter or longer times may be employed if desired.

In order for the process of this invention to operate successfully the pH of the aqueous dispersion should be at least 9. There is no critical upper limit to the pH except that under extremely strong alkaline conditions

leather deteriorates quite rapidly. Consequently, such conditions should obviously be avoided. Any alkaline material can be used to regulate the pH. Examples of suitable materials include alkali metal carbonates, alkaline earth metal oxides and hydroxides, alkali metal salts of carboxylic acids and ammonia.

The amount of organosilicon compound employed should be at least 10% of the dry weight of the hide. Larger amounts relative to the hide can be employed if desired. There is no critical upper limit to the amount of the organosilicon compound although for practical purposes large excesses should be avoided due to the expense of organosilicon compounds.

The temperature at which the operation of this invention is carried out is not critical. However, satisfactory results are obtained at room temperature and ordinarily there is no reason to vary therefrom.

For the purpose of this invention R can be any aliphatic hydrocarbon radical of less than 4 carbon atoms such as methyl, ethyl, propyl, isopropyl and allyl. The organosilicon compounds employed herein are best prepared by reacting the dialkoxysilanes of the formula



25 with vinyl and allyl glycidyl ethers in the presence of a platinum catalyst (i.e. chloroplatinic acid) at 80 to 120 C. Under these conditions the addition of the SiH to the vinyl or allyl group in the ether takes place to produce the compounds of this invention in which n is 2 or 3 respectively. Those compounds in which R is unsaturated are best prepared by an ester interchange between



35 and an unsaturated alcohol such as allyl alcohol. During the interchange methanol is given off.

After the hides of this invention have been tanned the resulting leather can be subsequently treated by any of the conventional processes which are employed to render leather suitable for fabrication. That is, the leather can be fat liquored with any of the conventional fat liquoring agents and it can be finished with any of the conventional finishing agents. Also, if desired, the leather can be rendered water repellent with any of the conventional leather water repellent agents, preferably with silicone water repellents.

The process of this invention can be carried out with any of the commonly employed animal hides such as horsehide, pigskin, sheepskin, goatskin, cowhide and the like.

The following examples are illustrative only and should not be construed as limiting the invention which is properly delineated in the appended claims.

## Example 1

A piece of limed, bated cowhide weighing 2744 g. (dry weight) was placed in 10 gallons of an aqueous solution having a .2 mol concentration of  $\text{Na}_2\text{CO}_3$  and containing 10% by weight  $\text{Na}_2\text{SO}_4$  based on the weight of the solution. The solution had a pH of 11. The hide was agitated in the solution at room temperature for 2 hours and then 880 g. of



65 was added and the agitation continued for 24 hours after which time the leather was removed and washed. The leather so produced had the following properties. The color was white, the shrinkage temperature was 82° C. and the leather was 96% undigested after the papain digestion test. The latter was run in accordance with

the procedure shown by F. G. Lennox and H. M. Forss, "Journal Society Leather Trades' Chemists," 36, 322 (1952). By contrast the untanned hide had a shrinkage temperature of 64° C. and was only 1.56% undigested after the above papain digestion test.

The leather was split and then divided into three portions. One portion (1) was fat liquored using an emulsion of a mixture of sulfonated sperm and neat's-foot oils (sold under the designation 1012W), said emulsion having a concentration of 6.5% oil. A second portion (2) of the leather was fat liquored with another emulsion of 1012W, said emulsion having a concentration of 9% oil. A third portion (3) was fat liquored with an aqueous emulsion of 4% by weight of a siloxane composed of a mixture of equal parts by weight of a dimethylpolysiloxane fluid and a methylpolysiloxane resin. The resin was composed of a copolymer of trimethylsiloxy groups and  $\text{SiO}_2$  units. In each case the resulting leather was flexible and pliable and suitable for use in the fabrication of articles.

Fat liquored leather (1) shown above was cut into 8 samples and each was immersed in a 15% solution of the siloxane water repellent shown in U.S. Patent Re. 23,879. The samples were tested for water penetration in accordance with the flex test shown in said patent. The average number of flexes before water penetrated was 6172. This compares with the commercially acceptable water penetration of 4000 flexes for leather treated with this silicone water repellent. This test shows that the white leather of this invention can be satisfactorily water repelled with commercially available silicone water repellents.

**Example 2.**

Equivalent results are obtained when the following organosilanes are substituted in the process of Example 1:



That which is claimed is:

1. A method of preparing leather which comprises contacting hide with an aqueous dispersion of an organosilicon compound of the formula



in which R is an aliphatic hydrocarbon radical of less than 4 C atoms and n is an integer of from 2 to 3 inclusive, at a pH of at least 9 until the hide is suitably tanned, the organosilicon compound being present in amount of at least 10% of the dry weight of the hide.

2. A method in accordance with claim 1 in which the organosilicon compound is



No references cited.

UNITED STATES PATENT OFFICE  
CERTIFICATE OF CORRECTION

Patent No. 2,970,881

February 7, 1961

Richard W. Alsgaard et al.

It is hereby certified that error appears in the above numbered patent requiring correction and that the said Letters Patent should read as corrected below.

Column 1, line 22, for "bleeding" read -- bleaching --.

Signed and sealed this 31st day of October 1961.

(SEAL)

Attest:

ERNEST W. SWIDER

Attesting Officer

DAVID L. LADD  
Commissioner of Patents  
USCOMM-DC